

May 1, 1934.

J. H. SWAN, 3D

1,957,368

PAPER MANUFACTURE

Filed Aug. 30, 1929

2 Sheets-Sheet 1



BY

INVENTOR  
Joseph H. Swan III  
Marechal and Rose  
ATTORNEYS

May 1, 1934.

J. H. SWAN, 3D

1,957,368

## PAPER MANUFACTURE

Filed Aug. 30, 1929

2 Sheets-Sheet 2



*INVENTOR*

Joseph H. Swan III  
Marshal and Noe  
ATTORNEYS

Patented May 1, 1934

1,957,368

# UNITED STATES PATENT OFFICE

1,957,368

## PAPER MANUFACTURE

Joseph H. Swan, 3d, Middletown, Ohio, assignor  
to The Gardner-Richardson Company, Middle-  
town, Ohio, a corporation of Ohio

Application August 30, 1929, Serial No. 389,424

8 Claims. (Cl. 91—68)

This invention relates to the manufacture of paper, and particularly to the manufacture of board adapted for use in the making of containers and the like.

5 One of the principal objects of this invention is to provide a paper or board which is grease proof and moisture proof, is sufficiently flexible and elastic to permit bending, is substantially odorless and tasteless, stands up well in use and 10 does not objectionably deteriorate on standing for considerable intervals of time, and is commercially economical.

Another object of the invention is to provide a method of forming such a grease proof paper or 15 board, which is simple, economical and highly effective, and which permits the continuous application of a composite coating with the formation of a product of good character.

Still another object of the invention is to provide 20 an apparatus for carrying out the above method.

Other objects and advantages of the invention will be apparent from the following description, from the accompanying drawings and 25 appended claims.

In the drawings in which like characters of reference designate like parts throughout the several views thereof,—

Fig. 1 is a partial diagrammatic side elevational view of apparatus constructed for carrying out the method of this invention;

Fig. 2 is a view similar to Fig. 1 disclosing another portion of the apparatus;

Fig. 3 is a plan view of the apparatus shown 30 in Fig. 1, certain parts being broken away and in section to illustrate the construction thereof;

Fig. 4 is a vertical sectional view taken on the plane of the line 4—4 of Fig. 2; and

Fig. 5 is a vertical sectional view on an enlarged scale of a container board made in accordance with this invention.

This invention is particularly applicable to the rendering of paper or board, such as container board, impervious to grease so that containers 45 made therefrom may be used for packaging greasy or oily substances which would otherwise penetrate through the package. When such a product is used for packaging foodstuffs, it is particularly desirable that the surface of the 50 container board be substantially tasteless and odorless. The coating should be of such character as to form an impervious layer on the surface of the board without pin holes which destroy the effectiveness of the coating, and it should be 55 sufficiently flexible and elastic to permit bending

of the board, such as is necessary in the formation of the box or container, without cracking. The coating should also be of a durable nature and one that will stand up well in use and will not objectionably deteriorate upon standing for 60 considerable intervals of time. In accordance with the present invention, a coated paper product is formed which is unusually efficacious in satisfying the above requirements.

Referring to the drawings which disclose a 65 preferred embodiment of apparatus constructed in accordance with this invention, a roll of paper to be coated is indicated at 10 carried by a suitable reel which is journaled at 11 upon a framework 12. The paper to be coated passes in a 70 travelling web indicated at 13 over suitable guide rolls 14 and 15 and thence passes in contact with the upper surface of roll 16 of a coating press. This coating press comprises also a lower roll 17 dipping within a trough 18 to which the coating 75 solution is uniformly supplied in any suitable manner. Rolls 16 and 17 are positively driven, and are mounted in adjustable bearings so that they can be vertically adjusted relatively to each other so as to contact at the nip with the desired pressure. In operation, rotation of the lower roll 17 within the coating solution serves to pick up a film of the coating material upon the surface of the roll. A portion of this film is transferred to the surface of the upper roll 16, 80 85 the amount or thickness of the film being regulated by adjusting the pressure of contact of the rolls 16 and 17, and this film is then transferred to the travelling web 13.

The coating composition applied at this point 90 comprises a rubber latex, a water solution of an oil insoluble adhesive such as sodium silicate, and an alkaline compound such as ammonia or sodium hydroxide adapted to maintain the coating in an alkaline condition. The rubber latex 95 is a relatively concentrated water solution or emulsion of the pure sap of the rubber tree in colloidal state. The addition of an oil insoluble adhesive, such as sodium silicate, to the rubber latex imparts superior characteristics of adhesiveness, thereby providing an excellent composition for this purpose. Rubber latex has qualities of elasticity and spreading ability and enables a relatively thin coating to be used with satisfactory covering power; it also functions very satisfactorily to lay any fuzz which may be protruding from the surface of the paper and covers up irregularities, such as pores and pinholes, of the surface. It is also a good moisture proofing and water proofing agent.

An alkali metal silicate provides a very satisfactory oil insoluble adhesive, and mixes satisfactorily with the rubber latex. Other oil insoluble adhesives such as casein, various animal 5 or fish glues or gelatine, may be used for this purpose. Other alkali metal silicates such as potassium silicate can be used in place of sodium silicate; but from the standpoint of economy the latter is preferred. The presence of an alkali 10 in the coating prevents deterioration of the same on standing and serves to increase the effective life of the coating.

In the preparation of the coating composition, the oil insoluble adhesive is made up in a relatively 15 concentrated solution. Thus where sodium silicate is used, a water solution containing in excess of about 20% sodium silicate is preferred. Satisfactory results may be secured with a solution containing from about 15% to 60% sodium 20 silicate by weight. The alkaline compound such as ammonia is added to either the rubber latex or the sodium silicate or both, and the solutions are then mixed. Satisfactory results have been secured with compositions containing from 10% 25 to 90% by volume of latex, the balance being primarily a water solution of sodium silicate of the above strength, this composition containing about 1% to 2% by weight on the total solids of an alkaline compound adapted to preserve 30 the alkalinity of the coating. Where the coating is used for a lower or base coat it is found preferable to provide in excess of 50% rubber latex by volume in order to give a base coating which has high flexibility and covering power.

35 As an example of a very satisfactory coating composition for the base coat which is applied to the paper or board, the following is mentioned: Sodium silicate solution of about 38% strength, and rubber latex containing about 38% by weight 40 of rubber hydrocarbons and the balance water and ammonia, are mixed in the proportions of about 60% or more by volume of rubber latex and 40% or less by volume of sodium silicate solution to form the liquid coating composition.

45 In accordance with the present invention, a composite grease proofing coating is provided on the surface of the paper or board, which composite coating is made up of upper and lower coats having different characteristics and which 50 are found to combine to give a superior resultant coating. The lower coating provides high flexibility and the upper coating provides high grease-proofness and moistureproofness, the composite coating resulting in a very satisfactory grease-proof and moistureproof sheet which can be 55 formed on a forming machine for manufacture into containers or the like.

The web 13 with the coating applied to the under-surface thereof at the coating press 16-17 then 60 passes with the uncoated surface in contact with the guide roll 20, and thence with the coated surface in contact with the surface of upper roll 21 of a second coating press. This coating press is constructed similarly to the coating press previously described and has a lower rotatable roll 65 22 dipping within trough 23, whereby a film of coating of the desired thickness is transferred from the lower roll 22 to the upper roll 21 and thence to the previously coated surface of the travelling web 13.

The upper layer of the composite grease proofing coating applied at this point comprises a polyhydric alcohol such as glycerine, an oil insoluble adhesive such as sodium silicate, and a suitable binder. The oil insoluble adhesive, such

as sodium silicate, has high grease proofing qualities, and also assists in securely binding the coating to the sheet. The addition of glycerine to the sodium silicate imparts characteristics of resiliency to the upper coating and tends to prevent cracking thereof when the board is bent in the formation of the container without impairing the greaseproofing character thereof, and also improves the spreading and covering power of the coating. Other polyhydric alcohols, for example glycols such as ethylene glycol, can be used with satisfactory results in substantially the same manner as glycerine. Other oil insoluble adhesives, such as casein, glues or gelatine, or other alkali metal silicates such as potassium silicate, can be used in place of sodium silicate.

With this coating containing an alkali metal silicate is preferably incorporated a binder, such for example as an oxidized starch, starch acetate or ground talc, flour, chalk and the like. A water soluble starch compound, such as an oxidized starch or starch acetate, are preferred due to ease of handling and superiority of results. Such starch compounds may be formed into a water solution and then added to the coating composition to provide a uniform and free-flowing coating which is readily applied at the coating press. Such a binder is found to improve the top coating, to make it more durable, and to prevent the possibility of the coating flaking in a dry atmosphere. In the preparation of the coating composition for this top coat, the alkali metal silicate is made up in a relatively concentrated water solution as is the case with the base coat above described. The oxidized starch is also made up into a suitable water solution by heating the starch compound in water such as by the introduction of steam. Satisfactory results have been secured with compositions containing from 15% to 40% by volume of glycerine, the balance being made up of a water solution of sodium silicate and the binder.

As an example of a very satisfactory coating composition for the upper coat, the following is mentioned: Sodium silicate solution of about 38% strength is mixed with glycerine and an oxidized starch solution in the proportions by volume of about 35% sodium silicate solution, 20% glycerine, and 45% starch solution containing about one pound of the soluble starch compound to a gallon of water.

The composite grease proofing coating thus produced has superior characteristics to a coating formed by merely a plurality of coats of a particular composition. The first or base coat provides a permanent non-deteriorating coat next to the sheet which acts as a protective coat to prevent the upper layer or coat from sinking into the sheet. The base coat provides unusual flexibility which is quite important in container board which is subjected to severe bending in the manufacture of the ultimate containers. This coating forming a flexible background for the overcoat, thus assists in preventing cracking of the overcoat upon bending of the board. The high percentage of a rubber compound such as rubber latex in the base coat acts as a water proofing and moisture proofing agent; and the spreading or covering power of this material together with its flexibility enables a substantially impervious coating to be formed with only a relatively thin film. This is materially assisted by the fuzz laying quality of the base coating. The upper layer or overcoat acts as a deodorizer of the base coat, and fills in any pores or pin holes

80

85

90

95

100

105

110

115

120

125

130

135

140

145

150

which may have been left by the base coating. The relatively high percentage of the oil insoluble adhesive, such as sodium silicate, gives an overcoat having high grease proofing qualities.

- 5 As many coatings as desired may be applied to the traveling web 13. Thus as shown, a third coating press comprising an upper roll 28 and a lower roll 29 dipping within a trough 30 is provided. If it is desired to apply only two grease proofing coats as above described, coating solution is not supplied to the trough 30. For the purpose of drying the coated web, drying blasts such as hot air blasts, are supplied to the coated surface of the web. As shown, a conduit 32 extends longitudinally beneath the coating machine from a point somewhat in advance of the first coating press to a point sufficiently removed therefrom to secure the proper drying of the web. This conduit is supplied with a drying fluid such 20 as air by means of a pump indicated diagrammatically at 33, the pump forcing air under pressure over suitable heating coils 34.

Intermediate the respective coating presses are upstanding ducts 35 and 36 which serve to direct 25 blasts of the heated air against the traveling web so as to dry the coating sufficiently to permit the next coat to be applied. The duct 35 discharges the heated air against the web opposite the area at which the web is supported against guide roll 30 20, while the duct 36 discharges against the web at the area where it is supported by guide roll 37. This arrangement gives the proper tensioning and surface contact of the web at the coating presses and also serves to support the web and 35 hold it adjacent the discharge of the ducts to secure satisfactory drying while minimizing danger of breaking the web. Beyond the coating presses a plurality of upstanding extending ducts 38 are provided which branch off from the conduit 32.

Each of the ducts 35, 36 and 38 is constructed similarly to that shown more particularly in Fig. 4. The conduit 32 is provided with a rectangular opening 39 over which is mounted the respective duct, the end walls of which diverge as indicated at 40 so that an upper outlet opening 41 is provided which extends across the full width of the web. The openings 39 in the respective ducts progressively increase in cross section from the duct 35 throughout the series to the duct at the end of the conduit 32 to thereby equalize the distribution of air discharged from the respective ducts. The duct closest to the pump 33 and at the point along the conduit 32 where the pressure 55 is highest thus has the smallest effective opening, and the ducts farther along have progressively larger openings in accordance with the pressure gradient throughout the conduit 32. Each duct is also preferably provided with a throttle valve 42 carried by journals 43 mounted in the end walls of the duct. Each valve 42 may be separately controlled by a suitable lever 44, or the levers may be connected by suitable linkage to secure their simultaneous actuation.

55 The web 13 after leaving the last coating press passes under a guide roll 45 and then travels unsupported above the discharge ports of the various ducts to subsequent treating apparatus. The pressure fluid not only serves to dry the web during its travel but also sustains it suitably spaced from the discharge of the ducts so that the coated side of the web does not contact with solid objects until it is substantially dry. The upper ends of each of the ducts are provided with a flat rim or flange 46 of smooth metal so as to provide a

flat supporting surface for the web when the machine is shut down or the web is being threaded through the machine.

In accordance with the present invention an overlying water insoluble wax coat is applied over the grease proof coating in order to protect the under grease proof coating and to provide a substantially odorless and tasteless outer surface. Very satisfactory results are secured with paraffin, beeswax, montan wax, or other well known insoluble waxes. From the standpoint of economy and ease of application paraffin is preferred for this purpose. The overlying wax coat not only protects the under grease proofing coat from exposure and deterioration, but also adds to the water proofness and moisture proofness of the coating, which is particularly advantageous in the packaging of deliquescent substances, such as crackers for example.

For the purpose of applying the top wax coat a coating press is positioned beyond the driers. This coating press comprises an upper rotatable roll 50 and a lower rotatable roll 51, the rolls being mounted in bearings which are vertically adjustable in a suitable frame work 52 so as to adjust the pressure of contact at the nip. The web 13 passes directly through the nip of rolls 50 and 51 with the undercoated surface in contact with the surface of roll 51 which in turn dips within a suitable trough 53 provided in the frame work 105 52. This trough may be supplied with a paraffin size solution, or may be supplied with paraffin or other wax which is maintained in a molten condition by suitable heating coils. Rotation of rolls 50 and 51 causes a thin film of paraffin to be 110 picked up on the surface of roll 51 and thus transferred to the coated web, the thickness of the film being limited by the pressure at the nip.

The presence of a suitable binder, such as a soluble starch compound, in the top layer of the 115 grease proof coating causes the top paraffin coat to adhere firmly to the coated web. The use of such a binder has a further advantage in assisting in the control of the amount of paraffin or other wax which is taken up by the sheet during 120 the application of this top wax coat. Thus it is found that the higher the percentage of soluble starch in the upper layer of the grease proofing coating, the more paraffin the sheet will take for the same roll pressure at the nip, and vice versa.

The sheet then passes from the final coating press through pressure rolls 55 and 56 carried in vertically adjustable bearings by the frame 52. These rolls are preferably constructed in the manner of calender rolls and are steam heated. A 130 high degree of pressure is used at these rolls, and the pressure together with heat serves to render the top wax coat fluid and spread it uniformly over the surface of the coated paper. The pressure rolls 55-56 also serve as a driving means 135 for drawing the paper through the machine. The coated paper then passes to further treating apparatus, or is wound upon a reel 57, or may be passed to suitable cutters and cut into sheets of desired size for the manufacture of containers.

If desired, the paper or board previous to the coating as above described, may be first subjected to a sizing treatment. The sizing treatment is useful in that it tends to prevent curling of the sheet after the coating is applied. Thus the 145 board, or the layer of the board forming the outer surface which receives the coating, may be a "hard sized" sheet, or one which has been made up from paper stock to which a sufficient quantity of size, such as rosin or paraffin size, has been 150

added as to materially retard the rate at which water or ink penetrates into the sheet. Very satisfactory results are secured by forming a sheet from paper stock to which rosin size has been 5 added at the beaters in the proportion of about 80 to 100 pounds or more of size to 1200 pounds of pulp. A sheet which will stand up for approximately five minutes or over in the water drop test, which means that water will not penetrate the sheet at that time, is satisfactory. Or 10 the sheet may be given a surface sizing by an application of a size to the surface of the formed web, using suitable conventional sizing materials such as above specified. The surface sizing may 15 be applied during the formation of the sheet prior to the application of the grease proofing coating. The sized paper is then supplied in roll form as indicated at 10 to the coating machine and the grease proofing coating is applied to the sized 20 sheet.

Referring to Fig. 5, a section through a preferred sheet or board is disclosed, which is found to be highly effective for use in containers for the packaging of greasy materials, and which 25 protects the materials from water and damp atmospheric conditions. The sheet comprises inner layers of ordinary board stock 60, with an intermediate layer 61 of asphalt material, such as an emulsion of asphalt and clay. The outer surfaces 30 of the board are formed of good grade liner stock, there being a bottom liner 62 and a top liner 63. One of the outside liners, such as the top liner 63, which is adapted to form the interior of the container and to receive the grease proof coating, 35 may be a hard sized sheet.

This board as above described may be formed on a conventional cylinder mold machine having a number of molds to form the various layers or plies of the sheet, these plies being brought together and united in the ordinary manner. Thus 40 a conveying felt of the forming machine passes first across a cylinder mold containing the bottom liner stock and forms a web, and then passes successively across cylinder molds provided with 45 board stock, asphalt emulsion, board stock, and finally top liner stock to form the complete built-up sheet of container board. The board as thus formed is then passed to the coating machine where the composite grease proofing coating is 50 applied, there being a lower or base coat of high flexibility indicated at 64 and an upper or overcoat of high grease proofing quality indicated at 55 65. A final overlying water insoluble wax coat 66 is then applied over the grease proofing coating. A container formed from this sheet is protected from water and moisture tending to penetrate from the outside into the interior of the 60 container by the intermediate asphalt layer and by the base coat 64, and is made effectively grease proof, water proof and moisture proof on the interior by the coating applied to the interior surface of the container.

While the forms of invention disclosed herein constitute preferred embodiments thereof, it is 65 to be understood that the invention is not limited to these precise forms, and that changes may be made therein without departing from the scope of the invention which is defined in the appended claims.

70 What is claimed is:

1. A paper product of the character described comprising a sheet having a composite grease-proofing surface, said sheet and composite surface being flexible to maintain the continuity of 75 said surface material against disruptive effects

during use, said surface comprising a lower layer including rubber latex and an oil insoluble adhesive, an upper layer including an oil insoluble adhesive and a binder, and an overlying top coat of a water insoluble wax, the binder being of such character as to modify the retention and adhering properties of the coated sheet for the water insoluble wax. 80

2. A paper product of the character described comprising a sheet having a composite grease-proofing surface applied thereto, said grease-proofing surface comprising a lower layer having high flexibility and including rubber latex and an alkali metal silicate, and an upper layer having high greaseproofness and including a polyhydric alcohol and an alkali metal silicate, said sheet and composite coating being flexible to maintain the continuity of said composite coating against disruptive effects in use due to bending and the like. 85

3. A paper product of the character described comprising a sheet having a composite grease-proofing surface applied thereto, said grease-proofing surface comprising a lower coat which is the dried deposit of a solution containing in 100 excess of 50% rubber latex by volume, the balance being primarily a water solution of an alkali metal silicate of a strength in excess of 20%; and an upper coat which is the dried deposit of a solution containing in excess of 15% by volume of 105 glycerine, the balance having a substantial proportion by volume of a water solution of an alkali metal silicate of a strength in excess of 20%, said sheet and composite coating being flexible to maintain the continuity of said composite coating against disruptive effects in use due to bending and the like. 110

4. A paper product adapted for formation into containers comprising a sheet having a composite greaseproofing surface applied thereto capable of 115 withstanding bending operations incident to formation into containers without destruction of the impervious character of said surface, said greaseproofing surface comprising a lower layer of high flexibility including a rubber material, and an upper coating layer of high greaseproofness including a polyhydric alcohol and a soluble starch compound, said sheet and composite coating being flexible to maintain the continuity of 120 said composite coating against disruptive effects in use due to bending and the like. 125

5. A paper product of the character described comprising a sheet having a greaseproofing surface applied thereto, said greaseproofing surface comprising a lower layer of high flexibility including a rubber material, and an upper coating layer of high greaseproofness comprising a polyhydric alcohol, an oil insoluble adhesive, and a binder, said sheet and composite coating being 130 flexible to maintain the continuity of said composite coating against disruptive effects in use due to bending and the like. 135

6. A paper product of the character described comprising a sheet having a composite greaseproofing surface applied thereto, said greaseproofing surface comprising a lower layer of high flexibility including a rubber material, and an upper coating layer of high greaseproofness including a polyhydric alcohol, an alkali metal silicate, and a soluble starch compound, said sheet 140 and composite coating being flexible to maintain the continuity of said composite coating against disruptive effects in use due to bending and the like. 145

7. A paper product of the character described 150

comprising a sheet having a composite grease-proofing surface applied thereto, said grease-proofing surface comprising a lower layer of high flexibility including a rubber material, and an upper coating layer of high greaseproofness including an alkali metal silicate and a soluble starch compound, said sheet and composite coating being flexible to maintain the continuity of said composite coating against disruptive effects in use due to bending and the like.

8. A paper product of the character described comprising a sheet having a composite grease-

proofing surface applied thereto, said grease-proofing surface comprising a lower layer of high flexibility including a rubber material, and an upper coating layer of high greaseproofness comprising a water soluble starch compound and an overlying surface layer of a water insoluble wax, said sheet and composite coating being flexible to maintain the continuity of said composite coating against disruptive effects in use due to bending and the like.

JOSEPH H. SWAN, III.

80

85

90

95

100

105

110

115

120

125

130

135

140

145

15

20

25

30

35

40

45

50

55

60

65

70

75